

W. F. GOLTRA.

METHOD OF PRESERVING WOOD FROM DECAY.

APPLICATION FILED JAN. 2, 1912.

1,047,404.

Patented Dec. 17, 1912.



Attest.  
F. Fisher  
J. C. Museum.

Inventor:  
W. F. GOLTRA  
By  
Fisher & Moore  
Atlys.

# UNITED STATES PATENT OFFICE.

WILLIAM FRANCIS GOLTRA, OF CLEVELAND, OHIO.

## METHOD OF PRESERVING WOOD FROM DECAY

1,047,404.

Specification of Letters Patent.

Patented Dec. 17, 1912.

Application filed January 2, 1912. Serial No. 668,914.

*To all whom it may concern:*

Be it known that I, WILLIAM FRANCIS GOLTRA, a citizen of the United States, residing at Cleveland, in the county of Cuyahoga and State of Ohio, have invented certain new and useful Improvements in Methods of Preserving Wood from Decay, of which the following is a specification.

This invention relates to a method of preserving wood from decay, and is applicable especially to such wood or timbers as have been more or less completely worked into shape for use, such as cross-ties, fence posts, piles and prepared timber and lumber somewhat generally and particularly such as is to be exposed to the deteriorating influences of the elements, of which wooden bridges are an example.

Assuming for the present description that railway cross-ties are the timbers to be treated, the process goes forward in the order indicated in the diagrammatic drawing herewith and the first step is steaming the ties.

Immediately upon arrival of the ties at the treating plant, they are transferred to narrow-gage tram-cars, and run onto tracks into the steaming cylinders A, and the cylinders hermetically closed. The ties are then subjected to live steam for a period varying from thirty minutes to four hours, depending upon the character and condition of the stock, such as thickness of the pieces, density of the wood, species of the wood, moisture content and the like, and a steam pressure of about fifteen pounds should be the maximum.

Steaming effects a great reduction of the time subsequently required for seasoning the wood, whether it be in a dry-kiln with heated air or by natural air-seasoning; and it dissolves and withdraws the juices and saps and prevents decay when subsequently dried. It also softens the outer surfaces and opens the pores of such timber as may have had a preliminary air-seasoning and which may have become "case-hardened", thus permitting rapid evaporation of the moisture contained in the interior of the timber and thereby preventing much of the checking and splitting which is so common in cross ties and timber generally while undergoing air-seasoning.

Experiments under varying conditions in-

dicate that large timbers, such as railroad ties, piling, etc., may be steamed at twenty pounds pressure for as much as four hours without material depreciation of strength, and it has been demonstrated that in wood subjected to live steam under pressure not exceeding twenty pounds for a time varying from thirty minutes to four hours, according to kind and thickness of wood, the coloring of the wood is distributed, equalized and improved and rendered approximately uniform.

When steaming sawed ties or lumber, the pieces should be piled on cross sticks, about one inch apart horizontally, so that the steam will have access to all surfaces. The steam pressure should be only a few pounds at the beginning and gradually increased to not exceeding twenty pounds at the end of the operation, so as not to heat the timber too suddenly, which might cause checking and splitting, an effect which frequently occurs when hot oil is introduced into the retort on cold ties.

The next step involves natural and gradual evaporation of the condensed steam or moisture from the timber by stacking the same in a yard for air-seasoning. Thus, the loaded tram-cars are then drawn out onto a transfer table C, which is run to one of the parallel yard tracks where the ties B are to be stacked. The tracks D are divided into parallel sets of three rails each, so that a standard gage locomotive crane can stand on the wider track of one set and unload narrow gage tram-cars standing on the narrower track of the other set.

The next step is to machine the ties. When the ties have sufficiently seasoned and are ready for further treatment, they are taken from the stacks, passed through gaining and boring operations and loaded directly on the tram-cars and carried to the ovens for the completion of the drying.

Most ties, whether sawn or hewn, are either bowed or winding, and in either case the rail base crushes down the wood at the highest contact point. The machining of ties obviates the necessity of gaining them before laying in the track, thereby effecting a saving in time and labor of section men. It also should be borne in mind that during the time the ties are air-seasoning some distortion in shape will occur, and if gained

mechanically after such seasoning they will have faces in the same plane. Thus, a tie when first properly seasoned, then gained and bored and then properly treated with 5 antiseptics, has received the most perfect protection possible at every point against the destructive agencies of decay and mechanical wear.

After the ties have been steamed, yard 10 dried and machined, they are transported to drying ovens E. Air-seasoning in itself is not sufficient to insure a good preparation of the ties for the impregnating treatment, and should therefore be completed in drying 15 ovens. An average of twenty-four hours is sufficient time to heat timbers, such as railroad ties through and through, and during this time the moisture content will be reduced three to four per cent. The high 20 temperature of the impregnating fluid when introduced into the retort is thus maintained when it comes into contact with the wood and the penetration is deeper and more perfect. Ties exposed to the weather immediately prior to treatment are often drenched 25 by heavy rains and absorb considerable water. This off-sets, in a great measure, the air seasoning and makes it quite impossible to obtain good results from such seasoning 30 alone. The rapidity with which the drying can be carried on after the material has received a preliminary steaming or air drying therefore depends upon several factors, such as species of the wood, its softness or density, size, mass, intended use and the manner 35 in which it is presented to the air in ovens. The time required in the oven to complete the drying of railroad ties which have undergone the several preceding steps of my 40 process is between eighteen and thirty hours, or an average of twenty-four hours.

The drying oven as a structure is preferably built of cement and masonry and corresponds in length and size to the length of 45 the impregnating retorts, and is heated by means of heating coils placed under or in the bottom thereof. Each oven is adapted to be operated independently of the other, so that when one or more ovens are being 50 charged the others are not affected. At the beginning the temperature of the ovens should be about 95° and gradually raised to 150° to 175° F. A maximum temperature of 236° F. may be attained with boiler pressure 55 of 100 pounds.

The transfer from the drying ovens is quickly made by means of the transfer table C which carries the tram cars loaded with the ties, and no appreciable amount of heat 60 is lost while making the shift from the said ovens to the impregnating retort.

After the timbers have remained in the drying ovens E a sufficient length of time the trams are drawn out onto transfer table 65 C and immediately run into the impregnat-

ing cylinder F for chemical treatment. The entire impregnating operation takes about 240 minutes or about four hours.

The first step is to produce a vacuum up to 14° and which should be attained within thirty to forty-five minutes. This is for the purpose of withdrawing some of the air from the cells and pores of the wood and inducing absorption of chemical. The vacuum having been on for sufficient time it is held while the chemical is allowed to flow into the cylinder, which it does very rapidly by the help of the vacuum and gravity, until the impregnating cylinder is completely filled, it being understood that the chemical 75 has been previously heated to a temperature of 175 degrees F. When the air pressure in the impregnating retort reaches the atmospheric pressure, as shown by a vacuum gage, an air valve with an overflow pipe attached 80 is opened to let air escape from the retort while filling. As soon as the fluid begins to flow in a full stream through the overflow pipe, indicating that the retort is full, the air valve is closed. When the cylinder is 85 filled and the air pipe closed, the pressure pump is put in action and kept working until a pressure of say 100 pounds per square inch is obtained. The more the chemical 90 penetrates into the wood the more the force pump has to be kept at work to maintain this necessary pressure, and the impregnation is considered complete when the manometer shows, for at least twenty minutes, that without further pumping the pressure 95 has remained stationary at 100 pounds—thus showing that the chemical is no longer penetrating into the wood. The duration of this phase of the operation varies from one to two hours, depending upon many factors, 100 such as species of wood, its physical structure, proportion of heartwood and sapwood, degree of seasoning, a size, mass and many other conditions. The treatment should, in all cases, be carried on to "refusal", which obviates the necessity for 110 sorting ties or timbers into numerous groups, and this is the only way to secure complete and thorough impregnation. The pressure should not exceed 100 pounds to 115 the square inch, as it is liable to injure the fiber of the wood.

When the timber has absorbed all the chemical it will take air is pumped into the cylinder from above and the solution driven 120 out below back into the storage tanks. The solution valves are then closed and a vacuum immediately created in the cylinder by means of the vacuum pump. This need not exceed 14°, and is held about thirty minutes 125 to allow the ties time to drip.

When the ties or timbers get dry enough to handle the vacuum is released and the dripping returned to the working tank from which it was originally drawn. This is 130

accomplished by a "blow-back" system or other suitable means.

The apparatus herein shown and described is claimed in my co-pending application 668,915 filed concurrently herewith.

A woodworking apparatus adapted to prepare the ties or timbers for further treatment as herein set forth is illustrated, for example, in Letters Patent of the United States, No. 582,915, of May 18, 1897, and which illustrates a machine for boring and trimming railroad ties.

What I claim is:

1. The method of treating railway ties and other timbers, consisting first in steaming the timber until the contained sap cells have been ruptured and the contents liberated; then drying the timber for a season in the open air and following this with artificial drying until practically perfectly cured, and then finally impregnating the timber with a suitable preservative.

2. The method of preparing railway ties to receive a liquid preservative consisting first in boiling the ties in live steam until the natural juices are expelled; then air drying in the open for a season; then gaining and boring the ties to prepare bearing surfaces for rails and holes for spikes, thereby permitting a thorough impregnation at points where ties are machined; then drying the ties in an oven until perfectly dried through and at the same time heating them to a receptive temperature for the preservative solution and finally impregnating the ties.

3. The method of treating railway ties consisting in first steaming the ties with live steam until the sap and natural juices are driven out of the ties; then air seasoning the ties for a season and following this with hot air drying under confinement, and while the ties are yet warm impregnating them with a preservative solution applied under pressure and continued to the point of refusal.

4. The method of treating timbers consisting in first liberating the sap and natural

juices in the timber by the direct application of live steam and at the same time filling the pores of the timber more or less with deposits from the steam; then eliminating the residual moisture by comparatively slow initial drying to avoid checking, and following this with kiln drying and finally while the timbers are still warm impregnating the same with a chemical solution under pressure to substantially the point of refusal.

5. A process of treating wood, which comprises the steps of steaming, air drying, and heat drying, in the order stated.

6. A process of treating wood, which comprises the steps of steaming, air drying, heat drying and impregnating with a liquid, in the order stated.

7. A process of treating ties, which comprises the steps of gaining and boring the same to form rail seats and spike holes, and to allow greater permeability in these portions than in the body of the ties, drying and thereafter impregnating with a suitable liquid.

8. A process of treating ties, which comprises the steps, of steaming the ties, gaining and boring the same to form rail seats and spike holes, and to allow greater permeability in these portions than in the body of the ties, drying the ties and thereafter impregnating with a suitable liquid.

9. An article of manufacture comprising a railroad tie substantially devoid of its natural sap and moisture, and having spike holes bored therein, and rail seats gained on its upper surface, said seats lying in substantially the same plane, and being impregnated with a suitable preservative, the impregnation at and near the rail seats being heavier than in the other parts of the tie.

In testimony whereof I affix my signature in presence of two witnesses.

WILLIAM FRANCIS GOLTRA.

Witnesses:

F. C. MUSSUN,  
E. M. FISHER.